

Jan. 21, 1947.

C. C. MARCH

2,414,474

RESILIENT ABRASIVE DISK

Filed June 3, 1944



Inventor  
By *Cecil C. March*  
Carpenter, Abbott, Gubler & Kinney  
Attorneys

## UNITED STATES PATENT OFFICE

2,414,474

## RESILIENT ABRASIVE DISK

Cecil C. March, St. Paul, Minn., assignor to  
Minnesota Mining & Manufacturing Company,  
St. Paul, Minn., a corporation of Delaware

Application June 3, 1944, Serial No. 538,577

5 Claims. (Cl. 51—195)

1

This invention relates to improvements in abrasive devices, and especially to improvements in abrasive-coated disks for detachable and renewable application to the grinding heads of rotary grinding machines. Grinding heads of this type are disclosed, for example, in the R. P. Carlton Patent No. 1,686,898 of October 9, 1928.

Coated abrasive products which, although useful also in various other forms, are of particular utility in the form of abrasive disks, have heretofore commonly been made with a composite backing comprising a layer of cloth bonded to a comparatively stiff but resilient sheet material such as vulcanized fibre (i. e. so-called fish fibre), with abrasive grains bonded to the exposed cloth surface. While animal glue has been used both as the combining adhesive for laminating the cloth to the fish fibre, for impregnating the cloth layer and also as the abrasive bond, more recently certain synthetic materials, especially phenol aldehyde resins which are capable of withstanding both the elevated temperatures sometimes developed in the disk during dry grinding, and also the solvent action of water as employed in wet grinding, have been used as the abrasive bonding coat and as a coating and impregnating material for the exposed surface of the cloth (further removed from the fish fibre) prior to the application of the making coat.

I have discovered that both of such structures, i. e. where glue impregnates the cloth and where phenol aldehyde resin impregnates the cloth layer, provide disadvantages and drawbacks in the disk structure, and in the utility of the disk as a whole, which I am able to overcome by a different structure of the elements of the disk, and especially by a change in the cloth layer in relation to the grit bonding coat. Also in a preferred embodiment of my disc structure, the bond which unites the stiff sheet of vulcanized fibre or the like to my cloth layer is a material quite different from that used to treat and impregnate the cloth (especially from the grit-coated side thereof).

An abrasive grain shows maximum cutting efficiency when it is securely anchored in a hard and firm bond so that it cannot be displaced to a less effective position by pressure against the workpiece which it is desired to abrade. It is therefore advantageous to use a hard and firm abrasive bond where an efficient cutting action is desired (as distinguished from a mere polishing action). The composite backing member of an abrasive-coated disk, to be satisfactory, must

5 also be strong and relatively stiff and at the same time suitably flexible, in order to transmit the rotary motion of the grinding machine from the central portion of the disk to the peripheral portion which contacts the workpiece and which performs the abrading action, and also to withstand necessary flexing while permitting the application of sufficient pressure of the peripheral portion of the disk against the workpiece so as to obtain effective cutting action of the abrasive grains on the workpiece. By the use of a hard and firm combining bond for laminating the cloth and stiff sheet of vulcanized fibre or the like (in the combination where my cloth layer has a presize or impregnating treatment with an elastic or yieldable material such as a vinyl butyral resin) I have found that I can improve the force which can be exerted upon the workpiece during the cutting or grinding operation without very appreciably affecting the ability of my disk to withstand rotation in use. My hard, firm combining bond, as used in my structure, has the effect of adding to the strength and stiffness of the fish fibre without greatly cutting down the ability of the disk to withstand flexing.

10 The known hard rigid and firm resin bonding agents have, however, an unfortunate tendency towards brittleness. Flat abrasive disks heretofore made with such resins, as the abrasive bond and impregnant for the cloth, are difficult to attach successfully to the grinding head of the rotary grinding machine, since even the slight depression or bending of the central portion of the disc by the retaining clamping bolt of the grinding head (such as illustrated in the previously mentioned Carlton patent) when the same is tightened in place is ordinarily sufficient to cause radial cracking, which accelerates subsequent failure of the disc. Even where mechanical means are available to avoid this difficulty, a further problem is encountered; in use, the peripheral portion of such a disk will break up rather rapidly, resulting in excessive loss of both 15 abrasive grains and bond, when subjected to the severe stresses encountered by pressure against the workpiece during use.

20 In order to avoid the difficulties encountered when using these hard and brittle resin materials, the substitution of various flexible bonding agents has heretofore been suggested for the abrasive bond or binder coat. Where these flexible materials are used as abrasive bonding agents, however, relatively inefficient abrading action is obtained, due largely to the ability of

the abrasive grains to be displaced into less effective cutting positions.

In one previously suggested method for the production of a disk structure, a resilient thermoplastic bonding material is applied as the combining agent between a sheet material, such as fish fibre or a fiber-reinforced resinous sheet, and a layer of cloth; a coating of a thermosetting resin is then applied as an abrasive bond to the uncoated cloth surface (thus also impregnating the cloth), followed by an application of abrasive grains, and by heat curing of the thermosetting resin to the hard rigid stage. During application, and to a further extent during the preliminary stages of heat curing, the thermosetting resin thoroughly impregnates the cloth from the grit-coated surface thereof; and, after curing is complete, this furnishes a hard rigid support for the abrasive grains, but it definitely limits the utility of the abrasive disk structure as a whole, as I have now discovered. Among other things, with this construction, the bonding qualities between the fish fibre and the cloth have, in general, been deficient, and other deficiencies have also been encountered, including inability of the disk satisfactorily to withstand repeated flexing.

I have found that much improved flexibility of an abrasive-coated disk may be secured, while still providing a strong and efficiently firm and sufficiently stiff and hard backing member, by properly positioning a relatively minor amount of flexible resilient material within my disk structure.

In my novel type of disk, I preferably bond a layer of cloth to a sheet of fish fibre by means of a heat-convertible synthetic resin, e. g. a thin layer of a phenol aldehyde resin, which is then cured to form a firm bond. I then coat and impregnate the exposed side of the cloth with an elastic, yieldable synthetic resin which may be comprised of polyvinyl butyral resin for example, in an amount sufficient to prevent any substantial penetration of the subsequently applied making coat into the cloth. I next apply an abrasive bonding or making coat of heat-convertible synthetic resin, and a layer of abrasive grains, to the treated cloth surface. Following this a sandsize coating is usually applied. The making and sandsize coats are suitably cured. The presence of the relatively thin cross-section of elastic, yieldable synthetic resin, in the cross-section of the composite backing most subject to bending and to tensile stress, affords this new abrasive device special advantages in utility, performance characteristics and durability.

A possible explanation of the unexpected effectiveness of this limited amount of flexible material in flexibilizing the composite product and in preventing cracking and "breakup" of the product during application and use may be as follows: In the application and use of abrasive products such as coated abrasive disks and belts, bending of the sheet is invariably in a direction to place the abrasive-coated surface farthest from the center of curvature. The stress set up during bending (i. e. transverse stress) is compounded of tensile and compressive stresses; thus the portion of the backing adjacent the back surface of a disk is placed under compression, while the outer or abrasive-coated side of the backing is placed under tension. Fibrous materials are best able to resist bending and tension when the stresses applied are equalized over the individual fibers; they are least able to resist such forces when

rigidly held together to an extent which will tend to shear or rupture the fibers. On the other hand, brittle fibrous materials, which when flexed or cracked are very low or entirely lacking in tensile strength, may be high in compression resistance. The separate constituents of the novel composite backing of this invention are therefore (based upon this explanation) seen to be so located as to utilize their most valuable qualities or characteristics, respectively. Since this is so, the thickness of the flexible resilient layer in particular may, if desired, be considerably reduced from previously accepted requirements.

An example of an abrasive disk with an embrittled cloth layer is shown by N. E. Oglesby Patent No. 2,333,035, granted October 26, 1943. As previously stated, however, my objective is almost the direct opposite; that is, I desire a disk where the layer of the backing which is adjacent to the making coat is tough, resilient and capable of withstanding bending, distortion and repeated flexing during use, without breaking up.

To quickly illustrate and explain my invention, reference is made to the accompanying drawing, in which:

Figure 1 is a representation (exaggerated as to size) of a vertical cross-section of a portion of a sheet abrasive article made according to the present invention;

Figure 2 is a perspective view of a disk formed of the sheeted abrasive material shown in Figure 1; and

Figure 3 is a plan view of the sheeted abrasive article of Figure 1, with layers successively broken away to show the construction.

Briefly, a layer or thickness of cloth 12 is bonded by a combining adhesive 11 to a sheet of tough, comparatively stiff and hard yet moderately flexible and resilient backing material 10, to form a composite backing. The exposed surface of cloth is treated (impregnated or presized) with a flexible resilient film-forming material 13. The impregnated surface of the cloth is then coated successively with a binder coat 14, one or more layers of abrasive particles 15 and lastly a sandsize coat 16. Preferred specific elements in this combined abrasive disk structure are illustrated by the legends on the drawing.

#### Example 1

Vulcanized fiber or fish fiber of ten mil (0.010 inch) thickness and weighing approximately 25 lbs. per ream (480 sheets 9" x 11"), which is a material well-known in the art (for example, see the Carlton Patent No. 1,686,898), is coated on one side with 13.6 lbs. per ream of a 95% solution of a heat-hardenable phenolic resin as a combining adhesive, and then combined with a cloth drills, having a thread count of 72 x 48 and a thickness of .017 inch, originally weighing one pound per 2.75 yards 27.5 inches in width, which has been kier boiled for removal of sizing, and which therefore weighs about 16 lbs. per ream. The concentrated, viscous resin solution slightly penetrates and impregnates the surface of the cloth, but in the main, leaves the cloth unimpregnated. After heating the laminated structure to remove the solvent and to set up or partially cure the combining adhesive, so that the two laminations will not be pulled apart during subsequent operations, the exposed cloth side of the combination backing is impregnated and presized with 12.75 lbs. per ream of a 24% solution of a thermoplastic flexible resilient, elastic film-forming material containing polyvinyl butyral

resin as a major ingredient, and the solvent is removed by evaporation. An abrasive bond, which may be a solution of a heat-hardenable phenolic resin, is next applied to the exposed surface of the impregnated cloth, followed by a layer of abrasive grains and (after intermediate removal of solvent and partial heat curing of the abrasive bond) by a final sandsize coating of a similar phenolic resin solution, and the composite structure is then subjected to a final heating and curing operation. Where a grit No. 24 aluminum oxide abrasive grain is to be applied, the abrasive binder or making coat may consist of 14.45 lbs. per ream of an 85% resin solution; the sandsize coat may consist of 22.65 lbs. per ream of an 80% resin solution; and 90.5 lbs. per ream of the abrasive grains may be used. (The proportion of sandsize adhesive to making adhesive varies considerably with the size of the abrasive grains.)

A strong, tough, efficient grinding or abrading device is thus obtained which can be fashioned into disks for detachable and renewable application to the rotary grinding heads of disk sanding machines, and which when in use will permit the application of relatively high pressures of the disk against the workpiece, while effectively resisting "breakup" or disintegration of the disk and while still maintaining efficient abrading qualities.

The presize solution called for by the present example is prepared by mixing the following ingredients in a churn until a homogeneous solution is obtained:

| Parts by weight                                                                                                                    |      |
|------------------------------------------------------------------------------------------------------------------------------------|------|
| Polyvinyl butyral ("Vinylite XYSG" produced and sold by Carbide and Carbon Chem. Corp., New York)                                  | 15   |
| Coumarone-indene resin (Cumar CX grade produced and sold by the Barrett Division of Allied Chemical and Dye Corporation, New York) | 15   |
| Tricresyl phosphate                                                                                                                | 10.5 |
| 2-ethoxy ethanol                                                                                                                   | 80   |
| Hydrocarbon solvent (a high solvency type containing aromatic fractions)                                                           | 50   |

Vulcanized fiber, or other suitable or equivalent stiff but resilient sheet material, may be used in various thicknesses, for example from 5 mils (0.005") to 30 mils (0.030") depending on the grit size of the abrasive grains, the pressure to be applied by the disk against the workpiece, the character of the workpiece, the weight and type of combining bond, and on other considerations.

Various suitable heat-setting resinous abrasive bonds and methods for their preparation and use have been known, as for example shown in the copending application of Byron J. Oakes, Serial No. 293,192, Patent No. 2,357,350. The use of such resins as combining adhesives, abrasive bonds, and/or as sandsize coatings is contemplated herein. Such resins may be carried to a desired viscosity and stage of reaction by preliminary heating, and may then be diluted and their viscosity reduced with solvents such as 2-ethoxy ethanol prior to application. Subsequent heating of the coated web removes the solvent and further firms up the resin to the required degree. The resins used as combining adhesive, abrasive binder (i. e. making coat), and sandsize coating may if desired be of the same composition. However, it is usually preferred to use resins which have been more completely reacted, or which are capable of reacting more rapidly at a given temperature, for the abrasive bond, and more particularly for the

sandsize, than for the previously applied combining adhesive, in order to obtain sufficient curing of the later coats without overcuring of the earlier coats. The final curing of the resinous bonds may be accomplished in successive stages wherein the temperature is gradually increased.

The amount of heat-reacting resin to be employed as the combining coat depends, at least in part, on the thickness and stiffness of the vulcanized fiber or other sheet material, and on the weight (or thickness) of the cloth. Where a thin, relatively flexible sheet material is employed, a heavy resin coat may be used to impart additional stiffness and strength to the combination backing. However, the amount and fluidity of the resin must not be so great as to allow it to penetrate or impregnate the entire thickness of the cloth portion of the backing. In general, it is found desirable to allow the combining adhesive to penetrate the cloth to a depth of about 10% of its thickness.

The amount of flexible resilient presize material used to impregnate the remaining thickness of the cloth portion of the combination backing may also vary within quite wide limits. For example, when using the vulcanized fiber and cloth specified in Example 1, advantageous results have been obtained with as low as 6.8 and as high as 28.3 lbs. per ream of the presize solution therein disclosed. These amounts approximate 10 and 50% respectively of the hard resinous combining bond of the example, when calculated on the solids basis. The lower weights of presize impart less flexibility, and furthermore have in some cases resulted in decreased adhesion of the abrasive bond to the surface of the backing, possibly due to blistering caused by the presence of air entrapped in the voids in the surface resulting from incomplete impregnation by the presize material. On the other hand, the higher weights of presize may impart undesirably high flexibility, and may also permit loss of abrasive, when the disk is in use, by lowering the strength of bond between abrasive bonding material and backing. In this case, the cloth is possibly so well filled by the presize that the abrasive bond material cannot obtain mechanical anchorage by penetration into the body of the cloth, or perhaps the increased thickness of the flexible resilient layer permits excessive deformation and resulting breakage and removal of the hard firm resinous abrasive bond when the abrasive-coated disk is placed in use.

It is obvious that different grit sizes of abrasive grains will require different amounts and viscosities of abrasive bond and of sandsize, as well as different weights of the abrasive grain itself; and such variations are contemplated in this invention.

#### Example 2

For the polyvinyl butyral base presize solution specified in Example 1 there is substituted an equivalent amount of the following formula:

| Parts by weight                                                                                                                   |     |
|-----------------------------------------------------------------------------------------------------------------------------------|-----|
| Polyvinyl butyral as in Example 1                                                                                                 | 37  |
| Liquid resinous plasticizer (hydrogenated methyl abietate; "Hercolyn," produced and sold by Hercules Powder Co., is such a resin) | 50  |
| Carbon black                                                                                                                      | 0.5 |
| 2-ethoxy ethanol                                                                                                                  | 185 |
| Xylool                                                                                                                            | 75  |

In this example, a liquid resinous plasticizer takes the place of both the liquid plasticizer and the coumarone-indene resin used in Example 1, and similarly advantageous properties are obtained in the finished abrasive sheet material.

In some instances, and particularly where heavy grit sizes require the use of highly viscous abrasive bonding material, it has been found desirable to apply a preliminary presize coat of a more dilute solution of the same or a similar abrasive bonding material. Thus in Example 1, a second presize consisting of 12.75 lbs. per ream of a solution of heat-hardenable phenolic resin of the same composition as the abrasive bond but containing only 65% solids is applied after the application and drying of the original thermoplastic flexible resilient film-forming presize. This second presize, by virtue of its improved fluidity, penetrates the voids of the treated cloth and thereby secures better adhesion to the cloth than would the heavier, less fluid abrasive bond if applied directly. The presize is dried, and partially cured by heating if desired, before the abrasive bond is applied to the backing.

#### Example 3

A flexible presize which may in some cases be substituted for the polyvinyl butyral presize compositions of the previous examples may be obtained by the inter-polymerization of vinyl acetate and 2-ethylbutyl maleate. Thus, 30 to 80 parts of monomeric vinyl acetate may be inter-polymerized with 70 to 20 parts of 2-ethylbutyl maleate, in a water dispersion and in the presence of a suitable catalyst according to methods well-known in the art, to produce a dispersion of 100 parts of tough, flexible, resilient, film-forming copolymer. This dispersion may be applied to the composite backing of Example 1 in place of the presize there described, and the abrasive sheet material completed as before, to produce an improved type of abrasive disk having useful properties.

#### Example 4

A plasticized or flexibilized heat-setting phenolic resin may in some cases be substituted for the flexible presize of Example 1, where somewhat less flexibility is sufficient. The following formula has been found to give good results:

| Parts by weight                        |      |
|----------------------------------------|------|
| Phenol-formaldehyde heat-setting resin | 42.5 |
| Diethylene glycol maleate              | 42.5 |
| 2-ethoxy ethanol                       | 7.5  |
| Water                                  | 7.5  |

The phenol-formaldehyde heat-setting resin may be of the same type as used for the combining adhesive and/or the abrasive bond. During the subsequent heating of the abrasive sheet, this resin also sets up or cures to a more advanced stage, but the presence of the diethylene glycol maleate renders the final product sufficiently flexible and resilient so that the abrasive sheet shows desirable improvement over the conventional type which contains no flexibilizing agent.

While the phenol-formaldehyde resin itself is here heat-setting, the final composite plasticized resin product is less rigid than would be the heat-set resin alone, and for the purposes of this invention is therefore equivalent to a thermoplastic resin.

Various other materials may also be used in some cases, either alone or in combination, as the flexible presize layer 13. Polymerized acrylates and methacrylates, and inter-polymers of

acrylates and methacrylates with other members of the same class or with other polymerizable materials such as alkyl fumarates or maleates, for example inter-polymerized methyl ethyl acrylate-*amyl* fumarate may be used, application being from solution in volatile organic solvent or from aqueous dispersion; suitable tackifying or otherwise modifying resins and the like may be added where necessary. Plasticized glutinous materials, such as animal glue plasticized with formaldehyde, may be employed; where such compositions are subject to the effects of moisture, or high temperature with high humidity, they may be "tanned" or rendered waterproof and heat-resistant by the action of aldehydes or other tanning agents. Drying oils or drying oil varnishes are also suitable for use as the flexible presize layer; thus a linseed oil varnish containing either the usual varnish resins, or preferably containing a rosin adduct formed by heating together one part of maleic anhydride with three parts of rosin, and containing also sufficient metallic driers to provide rapid and thorough drying of the varnish to a firm non-tacky but resilient film, may be used. Likewise alkyd resins, such as may be formed by condensation of polybasic acids with glycerol or glycol, may be used, as may also certain cellulose derivatives suitably plasticized and compounded, as with tackifying resins. Rubber, reclaimed vulcanized rubber, and synthetic rubber such as polymerized chloroprene, polymerized butadiene-styrene, polymerized butadiene-acrylonitrile, and the like, may also be suitably compounded and used for the saturation of the outer portions of the cloth layer to provide flexibility and resiliency of the composite structure. In general, any flexible, elastic, tough, yieldable, resilient, coherent material may be used which has the following properties:

1. It must not attack the cellulosic fibers of the cloth layer 12 so as to impair the strength thereof.
2. It must be able to withstand the temperatures encountered during heat curing of the abrasive bond and during the use of the abrasive disk, without becoming brittle and also without unduly softening.
3. It must have sufficient flexibility and be sufficiently yielding to permit equalization of stresses encountered in the outer portion of the cloth layer.
4. It must present a surface to which the abrasive bond coat will effectively adhere.
5. Its solution or dispersion in a volatile liquid vehicle must be capable of penetrating and impregnating the exposed and untreated portion of the cloth layer 12.

The improved abrasive-coated sheet of this invention thus consists, as will have become apparent from consideration of the specification, of a strong hard firm compression-resistant back layer, a strong hard firm abrasive layer, and an interposed flexible elastic yieldable resilient layer so situated that it provides maximum flexibility to the composite structure while still avoiding any unwanted softness. The hard firm and strong back layer is well-bonded and full-bodied, and is capable of transmitting a considerable amount of force from the central portion to the peripheral or abrading portion of a disk cut from the material without buckling or delaminating. The hard firm abrasive layer is well-bonded and strong so that the abrasive grains accomplish a maximum cutting action. The flexible resilient layer of the sheet, due

largely to its location in the composite structure as well as to its composition, provides desirable flexibility and freedom from "breakup" and disintegration, without limiting the cutting or abrading efficiency of the abrasive sheet or disk.

I claim:

1. A flexible abrasive disk of the coated abrasive type comprising a layer of vulcanized fiber, a hard firm thermoset phenol-aldehyde resin combining bond, a layer of cloth bonded to said vulcanized fiber by said combining bond and having the fibers adjacent said vulcanized fiber firmly incorporated within said combining bond, a layer of flexible resilient impregnant comprising polyvinyl butyral within the remaining portion and at the outer surface of said cloth, a hard firm strong thermoset phenol-aldehyde resin abrasive bond adherently bonded to said outer surface of said impregnated cloth, and a layer of abrasive grains bonded by the said abrasive bond.

2. A flexible abrasive disk of the coated abrasive type comprising a layer of vulcanized fiber of about 10 mil thickness and weighing about 25 lbs. per ream; a layer of cloth drills weighing about 16 lbs. per ream; a coating of thermoset hard and firm phenolic resin combining adhesive forming a firm, strong bond between said fiber and said cloth, and further forming a hard firm strong filling and unifying agent for not more than about 10% of the total thickness of said cloth; a layer of thermoplastic flexible and resilient cloth sizing material comprising polyvinyl butyral synthetic resin, forming an adherent, yieldable filling agent for that portion of said cloth layer furthest removed from the vulcanized fiber layer, said layer of cloth sizing material weighing approximately 3

lbs. per ream; and a further layer of thermoset hard firm and strong phenolic resin containing interspersed partly exposed abrasive grains, said layer being adherently bonded to said filled cloth layer.

10 5 15 20 25 30 35

3. A flexible abrasive disk of the coated abrasive type comprising a layer of vulcanized fiber, a hard firm thermoset synthetic resin combining bond, a layer of cloth bonded to said vulcanized fiber by said combining bond and having the fibers adjacent said vulcanized fiber firmly incorporated within said combining bond, a layer of flexible resilient impregnant comprising a thermoplastic synthetic resin having approximately the yieldability and elasticity of polyvinyl butyral resin within the remaining portion and at the outer surface of said cloth, a hard firm strong thermoset synthetic resin abrasive bond adherently bonded to said outer surface of said impregnated cloth, and a layer of abrasive grains bonded by the said abrasive bond.

4. A flexible abrasive disk as defined in claim 3, further characterized in that, in lieu of said layer of vulcanized fiber, there is employed, in the combination recited, any stiff but resilient, compression-resistant fibrous sheet having approximately the stiffness, toughness and resiliency of a sheet of vulcanized fiber of from 5 to 30 mils thickness.

30 35

5. A flexible abrasive disk as defined in claim 3, further characterized in that, in lieu of said layer of vulcanized fiber, there is employed, in the combination recited, any stiff but resilient, compression-resistant fibrous sheet having approximately the stiffness, toughness and resiliency of a sheet of vulcanized fiber of 10 mils thickness.

CECIL C. MARCH.